

# UNITED STATES PATENT OFFICE.

CLIFFORD RICHARDSON, OF NEW YORK, AND CHARLES N. FORREST, OF BROOKLYN, NEW YORK, ASSIGNORS TO THE BARBER ASPHALT PAVING COMPANY, OF PHILADELPHIA, PENNSYLVANIA, A CORPORATION OF WEST VIRGINIA.

## BITUMINOUS PAVING-BLOCK.

No. 358,116.

Specification of Letters Patent.

Patented May 7, 1907.

Application filed February 17, 1906. Serial No. 301,698.

*To all whom it may concern:*

Be it known that we, CLIFFORD RICHARDSON, residing in the borough of Manhattan, in the county of New York and State of New York, and CHARLES N. FORREST, residing in the borough of Brooklyn, in the county of Kings and State of New York, have invented certain new and useful Improvements in Bituminous Paving-Blocks, of which the following is a specification.

The invention has for its object the production of an improved paving block, which, while having the outward features and appearance of the ordinary asphalt paving blocks heretofore manufactured, is so proportioned internally as to possess greater durability when subjected to street traffic, while, at the same time, it insures constant and easily regulated conditions in the manufacture of such blocks and greater uniformity in the finished product than has heretofore been possible in the art.

The asphalt paving blocks heretofore manufactured have been composed, to the extent of ninety to ninety-five per cent of fine stone, known as crusher screenings, passing a screen of such a size that particles larger than one-quarter inch do not intentionally enter the product, and an asphalt or other bituminous cement to bind the mineral aggregate together. For convenience these screenings as they come from the crusher have been separated mechanically into two classes, viz: material fine enough to pass a ten mesh screen and that coarser than this, to be afterward combined into what has heretofore been considered suitable proportions for making the block aggregate. This manipulation does not affect the grading of either class of material, which remains the same as it left the crusher and which, while ostensibly divided into two sizes, contains a very large proportion, fifty per cent or more, of particles just a little smaller and just a little larger than ten mesh, with the result that it is not possible under the present practice, to produce with such particles an aggregate which will possess an appreciably greater compactness or freedom from voids or interstitial spaces when thoroughly compacted than ordinary sand. The reason for this is that the particles of about ten mesh size, or

lying in size between those not passing a twenty mesh and passing an eight mesh, are too large to fill satisfactorily the interstitial spaces or voids between the particles of four mesh stone, but on the contrary force these particles apart thereby increasing rather than diminishing the voids.

Now we have found that a much better mixture is secured by separating the crusher screenings in such a way that the particles retained on a twenty or thirty mesh screen and those passing an eight mesh screen are largely discarded. We then combine the particles smaller than twenty mesh screen, together with some dust as a filler, and those larger than eight mesh in such proportions as will result in an aggregate of the greatest density, having regard to the character of the fracture of the stone in hand, whether it be cubical, spall or of other form. These proportions usually approximate sixty-five per cent of the coarse and thirty-five per cent of the fine. In this way we secure an aggregate of great stability and compactness containing but from twelve to fifteen per cent of voids, whereas the same screenings without the advantage of the manipulation developed by our invention will contain a much larger per cent of voids. We have found further that even greater uniformity may be secured by eliminating entirely the material known as crusher screenings, which is far from uniform in the amount or size of individual particles, and possesses the usual irregularities of any by-product, and instead employing clean crushed stone, consisting of particles which will pass a three-quarter mesh screen and be retained on an eight mesh screen. This we preferably separate into two or more classes, such as those particles passing respectively a four mesh, two mesh, and three quarter inch screen, depending upon the dimensions of the block it is proposed to make. We then recombine these materials in definite proportions with a fine sand (ranging from ten mesh to one-hundred mesh), and an impalpable mineral or other powder finer than two-hundred mesh, graded according to United States Letters Patent No. 607,884, granted Clifford Richardson, July 26th, 1898. In this way, an aggregate may be produced of greater

compactness than is possible by any other method of selection heretofore practiced in the art for the selection of an aggregate for the production of asphalt paving blocks.

5 To practice our invention any hard crushed stone suitable for the purpose is taken and divided by screening into particles which will be retained on a one-eighth mesh screen and pass a one-quarter mesh screen, 10 and particles larger than one-quarter mesh but smaller than one inch mesh. We also take clean fine sand of the grading mentioned in Richardson's Patent No. 607,884, above referred to, and an impalpable mineral or 15 organic powder the particles of which will pass a two-hundred mesh screen. The drying, storage and handling of all of these materials is done in the usual manner and with aid of the machinery well known in the 20 art. Definite proportions of these materials, which are determined by weight, are then worked together in a suitable apparatus until thoroughly mixed, when an amount of asphalt cement or other suitable bituminous 25 binding material is introduced to fill the remaining voids and to coat as well the surface of each individual particle of the mineral aggregate so that when the resultant product is compressed in the block press a homogeneous 30 block with a smooth surface is produced resembling in compactness a solid block of stone. It is apparent that the size of the largest particles in this improved aggregate will be influenced as before stated by the 35 size of the finished block it is proposed to make, and while it is not our intention to be limited as to the dimensions of any block, we have particular reference to the sizes which have heretofore been found convenient for manufacturing and handling. For instance, in a block three inches thick, five inches wide, and twelve inches long, it is not desirable to use stone larger than 40 will pass a three-quarter mesh screen, and in smaller sizes the maximum may be reduced to that passing a one-quarter inch or one-half inch mesh screen. It is also apparent that the degree of pressure employed in molding the blocks will influence the appearance 45 of the same, but in the art it is not practicable to exceed a certain pressure (and indeed the manufacturer is frequently confined to certain minimum or maximum limits in this respect by the specifications of the consumer 50 to whom the finished product is to be supplied), and with such practice we mention the following proportions as suitable for illustrating our invention when applied to a block three inches thick, five inches wide and twelve inches long:—stone, passing three-quarter inch and retained on one-half inch mesh screen, twenty per cent; stone, passing one-half inch and retained on one-quarter inch mesh screen, twenty-eight per cent; stone passing one-quarter inch and retained

on one-eighth mesh screen, eight per cent; finer material passing ten and retained on two-hundred mesh screen, twenty-five per cent; dust or filler passing two-hundred mesh screen, twelve per cent; and bituminous binding material, seven per cent. Of the above the sand or finer material passing ten and retained on two-hundred mesh screen (of which twenty-five per cent is mentioned), should have the following grading or as near to it as local sand supplies may permit:—

|                       |     |    |
|-----------------------|-----|----|
| Passing 100 mesh, 17% |     |    |
| " 80                  | 17% | 80 |
| " 50                  | 30% |    |
| " 40                  | 13% |    |
| " 30                  | 10% |    |
| " 20                  | 8%  |    |
| " 10                  | 5%  | 85 |

But although we have specified with exactness this preferred grading according to our invention, we do not limit ourselves to this grading, for similar advantages may be secured by other mixed aggregates employing the principle of our invention. This principle is briefly this, that having regard to the maximum sizes of stone to be employed, but assuming about one-half or three-quarter inch as the maximum, there should be a marked diminution or approximate elimination of the sizes of material which lie between the one-eighth inch and the one-twentieth inch sizes.

In the claims which follow, we use the phrase "a mineral aggregate of crushed screenings." This should be understood to mean an aggregate such as is produced by screening an ordinary crusher run of stone through a screen of about three-quarters of an inch in mesh, containing all sizes of stone from an impalpable powder up to particles just passing such a mesh. While such screenings may vary to a certain extent according to the nature of the stone, or the kind of crusher employed, yet there will always be present a fairly constant proportion of materials of all sizes, and it is our discovery that in employing such crushed screenings for the purpose specified, there should always be eliminated a considerable proportion of the particles which lie between the eight mesh and the twenty mesh screen in order to secure the desired density of the "aggregate."

Having thus described our invention, we claim:—

1. A paving block composed of bituminous binding material and a mineral aggregate of crushed screenings running from about three-quarters of an inch down to impalpable powder with substantial depletion of the particles which pass a one-eighth mesh screen and are retained on a twenty mesh screen, substantially as specified.
2. A paving block composed of a bitumi-

nous binding material, and a mineral aggregate of crushed screenings not larger than three-quarters of an inch in size, and from which the excess of particles which pass a 5 one-eighth mesh screen and are retained on a twenty mesh screen are excluded, substantially as specified.

3. A paving block composed of a bituminous binding material, and a graded mineral aggregate composed of over 50% screened stone definitely graded from about three-quarters of an inch down to particles retained on a one-eighth mesh screen, and the balance of fine sand and dust graded, substantially as 10 specified.

4. A paving block composed of a bituminous binding material and a graded mineral aggregate of which approximately 65% lies between three-quarters of an inch and one-eighth of an inch in size, and the balance of 15 which passes a 20 mesh screen, substantially as specified.

5. A paving block composed of a bitumi-

nous binding material, and a graded mineral aggregate of which approximately 65% is 25 between three-quarters, and one-eighth of an inch in size, and the balance finer material graded substantially as follows:—

|                  |     |    |
|------------------|-----|----|
| Passing 100 mesh | 17% | 30 |
| " 80             | 17% |    |
| " 50             | 30% |    |
| " 40             | 13% |    |
| " 30             | 10% |    |
| " 20             | 8%  | 35 |
| " 10             | 5%  |    |

In testimony whereof, we have hereunto signed our names, at New York city in the State of New York this 15th day of February 1906.

CLIFFORD RICHARDSON.  
CHARLES N. FORREST.

Witnesses:

RICHD. H. BARKER,  
M. P. ENNIS.